

# UNITED STATES PATENT OFFICE.

CHARLES H. SNYDER, OF BALTIMORE, MARYLAND.

## COMPOSITION FOR GRINDING AND POLISHING.

No. 841,908.

Specification of Letters Patent.

Patented Jan. 22, 1907.

Application filed March 21, 1906. Serial No. 307,294.

*To all whom it may concern:*

Be it known that I, CHARLES H. SNYDER, a citizen of the United States, residing at Baltimore, in the State of Maryland, have invented new and useful Improvements in Compositions for Grinding and Polishing, of which the following is a specification.

This invention relates to an abrasive compound and to a wheel or other tool made of the compound, particularly adapted for grinding and polishing metal and substances, especially hard metals, such as steel, chilled iron, and the like.

The object of the invention is to form an improved wheel or tool characterized particularly by extreme hardness and rapid-cutting qualities, by porosity, by freedom from glaze, by durability, and by cheapness of construction.

The ingredients and proportions thereof used in making the composition for a wheel or tool are as follows: granulated or pulverized rock, six parts; red lead, two parts; sodium silicate, one part; and sawdust, one part. The rock referred to may be selected from the hardest and most refractory minerals obtainable, although it may be stated that emery cannot be used because it will not stand the high temperature to which the composition is subjected, as hereinafter explained. I use particularly a form of rock which so far as I know can be found only in one place and the chemical composition of which is not at this time known to me, al-

though I have been informed that it is a form of crystallized carbon, and I have applied thereto the name of "carbonate rock." This rock is capable of being granulated and pulverized to many degrees of fineness, and it does not lose its granular or sharp nature even when subjected to a high degree of heat. It is therefore particularly well adapted for use as the basis of an abrading tool. The invention, however, is not limited to this particular form of rock; but any mineral or substance having similar qualities may be substituted.

In making a wheel, for instance, the granu-

lated or pulverized rock of the desired degree of fineness is mixed with the other ingredients above mentioned to form a paste or plastic mass which can be molded. This is placed in a mold of desired shape and allowed to dry for a few hours. The wheel is then burnt in a kiln raised to a temperature of 900° Celsius. The sodium silicate or water-glass is used merely to make the composition plastic, so that it can be molded. The red lead is used as a binder. The sawdust is used to make the pores. The firing burns out the sawdust and the water-glass and leaves a hard wheel of gritty quality which will not glaze. If the mixing be well performed, the wheel will be of uniform hardness throughout. The porous quality acquired from burning out of the sawdust serves to prevent the wheel from glazing and has the further advantage that when used wet it will absorb and hold water. The sawdust is pulverized to a degree suitable for the kind of wheel being made. A coarse wheel—that is, a wheel having coarse granulated rock—requires finer sawdust to produce the desired result, while a wheel of fine or pulverized rock is best formed with coarser sawdust. A wheel formed of the composition is preferably supplied with a central core of metal or wood. As a result of the high temperature to which it is subjected, the wheel becomes hard and non-breakable by speed and can be used either wet or dry and will not burn the work when used wet.

I claim—

An abrading-tool formed of pulverized rock, red lead, sodium silicate and sawdust mixed together and subjected to heat sufficient to burn out the sodium silicate and the sawdust.

In testimony whereof I have signed my name to this specification in the presence of two subscribing witnesses.

CHARLES H. SNYDER.

Witnesses:

M. R. KUNSMAN,  
GEO. E. TEW.